

## UNITED STATES PATENT OFFICE.

ALAN KISSOCK, OF LOS ANGELES, CALIFORNIA, ASSIGNOR TO CARL M. LOEB, OF NEW YORK, N. Y.

## PROCESS OF PRODUCING MOLYBDATES.

No Drawing.

Application filed April 1, 1924. Serial No. 703,533.

*To all whom it may concern:*

Be it known that I, ALAN KISSOCK, a citizen of the United States, residing at Los Angeles, in the county of Los Angeles and State of California, have invented a new and useful Process of Producing Molybdates, of which the following is a specification.

This invention is a process for producing iron molybdates, which may be used in the manufacture of alloy steel, or for other purposes.

Objects and advantages of the invention are set forth in part hereinafter and in part will be apparent herefrom to those skilled in the art. The invention consists in the steps, sequence of steps, and processes hereinafter described.

One of the principal objects of the invention is to provide a process whereby there is produced direct from the ore or ore concentrate a finished product suitable for use directly in the steel furnace in the manufacture of alloy steel, and at a great reduction of cost and increase of efficiency over processes heretofore known.

The invention consists essentially in subjecting molybdenum and iron containing materials to an oxidizing roast, and at a temperature sufficient to cause them to split up and combine to form iron molybdate.

Using molybdenite, a commonly occurring sulfide ore of molybdenum, and iron oxide, the probable reaction is:



In this reaction, the ferrous oxide is oxidized to the ferric state, and the molybdenum is probably oxidized to the trioxide; although under some conditions molybdenum trioxide is volatile, there is no escape of molybdenum trioxide in this reaction; evidently it exists only for an instant, and immediately combines with the ferric oxide before it has time to escape as the trioxide. All the molybdenum appears as ferric molybdate.

Using molybdenite and iron pyrites, the probable reaction is:



or expressed in two stages:



or



In these reactions also, the molybdenum apparently exists as the trioxide only for an instant, because no trioxide escapes during the process. As in the first case, all the molybdenum appears as ferric molybdate.

The reacting materials are first roasted at a temperature of about 5-600° centigrade, which is gradually increased until the reaction is complete at about 1000° centigrade.

Certain naturally occurring ores of molybdenum, such as molybdenite, already contain iron, usually as the sulfide or oxide. If there is sufficient iron already present in the ore, it may be subjected to the oxidizing roast without the addition of any iron, or with the addition of only a sufficient amount of iron to bring the iron content to the proper point. This utilization of a naturally occurring ore containing both iron and molybdenum to produce iron molybdate without adding any more iron, or adding only sufficient iron for the purposes of the reaction, is a very important feature of this invention, because of the evident economy.

The theoretical proportions of iron and molybdenum are one part by weight of molybdenum to 0.4 part by weight of iron. If the naturally occurring ore does not contain sufficient iron, more may be added, as the oxide or sulfide, to bring up the iron content to the proper point.

The molybdenite ore which sometimes contains only 1% molybdenite, or the mixture of molybdenum and iron ore, is first concentrated so as to contain about 80% of molybdenite. Flotation or other known

processes may be used to effect this concentration.

In carrying out the process with molybdenite and iron pyrites, about 100 pounds of 80% molybdenite concentrates (containing no iron) is mixed with about 50 pounds of iron pyrites (containing about 82.56%  $FeS_2$ ) and the mixture roasted at about 5-600° C. for about one hour, thereafter gradually increasing the temperature and finishing at about 1000° C. for fifteen minutes.

In carrying out the process with molybdenite and an oxide ore of iron, about 100 pounds of 80% molybdenite (containing no iron) is mixed with about 30 pounds of iron ore containing 82.27%  $FeO$ , and the mixture roasted at about 5-600° C. for about one hour, thereafter gradually increasing the temperature and finishing at about 1000° C. for fifteen minutes.

These figures, it should be understood, are merely illustrative and not restrictive of the invention.

In a copending case filed by the same applicant on September 19, 1922, Serial No. 589,240, is disclosed a process for making calcium molybdate by subjecting molybdenum and calcium containing materials to an oxidizing roast, the preferred calcium containing material being calcium carbonate.

While this process is particularly applicable to producing iron molybdate, it is intended to cover the chemical equivalents of iron in the reactions noted above.

I claim as my invention:—

1. The process of producing molybdates, comprising subjecting a mixture containing molybdenum and iron to an oxidizing roast.
2. The process of producing iron molybdate, comprising subjecting a mixture of an ore of molybdenum and an ore of iron to an oxidizing roast.

3. The process of producing iron molybdate, comprising subjecting a molybdenum containing material to an oxidizing roast in the presence of iron.

4. The process of producing iron molybdate, comprising subjecting molybdenite to an oxidizing roast in the presence of an iron supplying material.

5. The process of producing iron molybdate, comprising subjecting molybdenite to an oxidizing roast in the presence of iron oxide.

6. The process of producing iron molybdate, comprising subjecting a mixture of molybdenum sulfide and iron sulfide to an oxidizing roast.

7. The process of producing iron molybdate, comprising subjecting an ore already containing molybdenum and iron to an oxidizing roast.

8. The process of producing iron molybdate, comprising subjecting an ore containing about 80% of molybdenite to an oxidizing roast in the presence of an iron supplying material.

9. The process of producing iron molybdate, comprising concentrating an ore already containing compounds of molybdenum and iron, adding more iron supplying material if necessary, and subjecting the mixture to an oxidizing roast.

10. The process of producing ferric molybdate, comprising subjecting a molybdenum containing material to an oxidizing roast in the presence of an iron supplying material.

11. The process of producing ferric molybdate, comprising subjecting a mixture of a molybdenum containing material and ferrous iron to an oxidizing roast.

In testimony whereof, I have signed my name to this specification.

ALAN KISSOCK.